

## 1

2,925,386

## MINERAL OIL BASE LUBRICANT

Wilhelm Dietrich, Hans-Joachim Mertens, and Fritz Wetter, Marl, Westphalia, Germany, assignors to Chemische Werke Huls Aktiengesellschaft, a corporation of Germany

No Drawing. Application August 4, 1953  
Serial No. 372,394

Claims priority, application Germany August 25, 1952

## 2 Claims. (Cl. 252—47.5)

It is known that in general mineral lubricating oils cannot be improved or can be only slightly improved with respect to their extreme pressure lubricating properties by the addition of aliphatic and aromatic nitro compounds including those which contain a halogen.

Mineral lubricating oils can however be improved with respect to extreme pressure lubricating properties by the addition of elemental sulfur. A greater resistance to loading at high pressure can be conferred upon gear and cutting oils by treating the corresponding mineral oils with sulfur. It has been proposed to add to mineral lubricating oil the sulfur containing products obtained by treating fats and animal and vegetable oils with sulfur. Such sulfur-containing mineral oils are however often corrosive and their extreme pressure lubricating properties although somewhat improved are not up to present day requirements.

It has been found that mineral oil base lubricants which contain both organic nitro compounds and oil soluble di- or poly-sulfides of xanthogenates hereinafter referred to as multi-sulfides of xanthogenates show a distinct improvement of their extreme pressure lubricating properties.

The expression "lubricants having a mineral oil base" includes not only true mineral oils but also the corresponding lubricant greases.

Suitable organic nitro compounds are for example, m-dinitrobenzene, bromodinitrobenzene, chloronitrobenzene,  $\beta$ -dinitrophenol and their C-alkyl derivatives and mixtures thereof and other nitro compounds including nitroparaffines, nitronaphthalenes and nitronaphthols, this enumeration being merely illustrative and not limitative.

The oil soluble multi-sulfides of xanthogenates are compounds of the general formula



in which R stands for alkyl, cycloalkyl, aralkyl, aryl and heterocyclic groups which may be straight chain or branched or saturated or unsaturated and may contain metal atoms such as tin or zinc. X stands for oxygen or sulfur and n means a figure from 0 to 5 or even greater.

Disulfides of xanthogenates are obtainable, as is well known, from xanthogenates by treatment in aqueous solution with oxidizing agents such as hydrogen peroxide, persulfates or hypochlorites, while for the production of the polysulfides, for example, the alkali metal salts of di- and trithiocarbonic acids are reacted by a well known process with sulfur chloride.

Suitable multi-sulfides of the said formula are e.g. dibutyl-, dipropyl-, diethylhexyl xanthic acid disulfide, diethylxanthic acid tetrasulfide.

The amount of nitro compound and multi-sulfide of xanthogenate and the particular compound to be used depend upon the purpose for which the resulting lubricant is to be used. In general the addition of nitro compound amounts to only a small fraction (up to one

## 2

tenth) of the addition of multi-sulfide, of which latter, depending upon the extreme pressure lubricity required, amounts within the range from 0.5 to 10% by weight calculated upon the weight of the pure lubricant are used.

5 The new lubricants, containing the nitro compounds and the multi-sulfides of xanthogenates, show no loss in weight due to corrosion at normal temperatures and only insignificant loss in weight due to corrosion at elevated temperature and after a long time of metals such as brass, bronze and copper. The lubricants which have been improved by the described additions of nitro and multi-sulfide compounds may be further improved by other well known additions for the improvement of extreme pressure lubricity, viscosity, solidification point, 15 foaming resistance and resistance to oxidation.

Testing of the extreme pressure lubricating properties of mineral lubricating oils with additions of the nitro and multi-sulfide compounds by the generally used four ball apparatus (VKA) and method described in the publication "01 und Kohle," 1944, pages 19-23, shows that with additions of 0.1 to 0.25% of the organic nitro compounds together with from 1 to 2.5% of the multi-sulfides of xanthogenates permits the application of loads of from 400 to 1000 kg. before a welding or freezing of 20 the balls occurs.

25 The invention is further described and illustrated in and by the following specific examples.

## Example 1

30 A spindle oil having a VKA value of less than 150 (density  $15/4^{\circ}=0.9024$ , viscosity at  $20^{\circ} C.=8.40^{\circ} E.$  and at  $50^{\circ} C.=2.47^{\circ} E.$ , viscosity index=115, solidifying point=-17° C.) was not improved with respect to its extreme pressure lubricity by the addition of 0.25% 35 of dinitrophenol. By the addition of 2.5% of dibutylxanthic acid disulfide the VKA value was raised to 340. The addition of both 0.25% of dinitrophenol and 2.5% of the dibutylxanthic acid disulfide raised the VKA value to 440.

## Example 2

40 To a mineral oil of average viscosity having a VKA value of 150 (density  $15/4^{\circ}=0.78$ , viscosity at  $20^{\circ} C.=47.2^{\circ} E.$  and at  $50^{\circ} C.=8.49^{\circ} E.$ , viscosity index=104, solidifying point=-12° C.) 2.5% of dibutylxanthic acid disulfide was added. The resulting lubricant had a VKA value of 480. By the further addition of 0.25% of  $\beta$ -dinitrophenol the VKA value was increased to 950. The addition of 0.25% of the  $\beta$ -dinitrophenol alone to the 45 pure mineral oil did not produce any improvement of the extreme pressure lubricity.

## Example 3

45 A lubricating oil, of a viscosity at  $50^{\circ} C.=20^{\circ} E.$  and a VKA value of 160-180 shows after the addition of 2.5% dipropylxanthic acid disulfide a VKA value of 360, which raises after the addition of 0.15% 6-chloro-2,4-dinitrophenol up to a value of 440. The addition of 60 6-chloro-2,4-dinitrophenol alone to the pure lubricating oil did not produce any improvement of the lubricity.

The mixing of the said pure lubricating oil with 2% diethylxanthic acid tetrasulfide improves the VKA value of the oil up to 440-460, by the further addition of 0.2% 2,4-dinitrophenol a lubricating oil with the VKA 65 value of 550-600 will be obtained.

The mixing of the said pure lubricating oil with 5% diethylhexylxanthic acid disulfide gives a lubricating oil with a VKA value of 500, which will be improved up to 600-650 by the further addition of 0.15% 6-bromo-2,4-dinitrophenol.

70 The multi-sulfides of a xanthogenate as well as the organic nitro compounds employed in the above ex-

amples may be substituted one with another in similar amounts and with similar results.

We claim:

1. A lubricant comprising a mineral oil base, 0.05-1% of an organic nitro compound selected from the group consisting of nitroparaffines, dinitrobenzenes, dinitrophenols, nitronaphthalenes, nitronaphthols and their halogens and C-alkyl derivatives, and 0.5-10% of an oil soluble multi-sulfide of a xanthogenate which is a member of the group of compounds of the general formula

10



in which R is a member of the group consisting of alkyl,

cyclo-alkyl, aralkyl and aryl, X is a member of the group consisting of sulfur and oxygen and  $n$  means a figure from 0 to 5, the ratio of said nitro compound to said oil soluble multi-sulfide being not more than 1 to 10.

5 2. A lubricant as defined in claim 1 in which the multi-sulfide of a xanthogenate is dibutylxanthic acid disulfide.

References Cited in the file of this patent

UNITED STATES PATENTS

- |           |                      |                |
|-----------|----------------------|----------------|
| 2,094,097 | Downing et al. ----- | Sept. 28, 1937 |
| 2,250,545 | Mikeska et al. ----- | July 29, 1941  |